

## UNITED STATES PATENT OFFICE.

GEORGE D. VAN ARSDALE, RUSH T. SILL, AND HARLEY A. SILL, OF LOS ANGELES,  
CALIFORNIA.

## METHOD OF PRODUCING MOLYBDENUM AND MOLYBDENUM COMPOUNDS.

No Drawing.

Application filed November 6, 1922. Serial No. 599,430.

*To all whom it may concern:*

Be it known that we, GEORGE D. VAN ARSDALE, RUSH T. SILL, and HARLEY A. SILL, citizens of the United States, residing in 5 Los Angeles, county of Los Angeles, State of California, have jointly invented certain new and useful Improvements in Methods of Producing Molybdenum and Molybdenum Compounds, of which the following is 10 a specification.

This invention has for its general object the provision of an improved method of extracting molybdenum from its ores, concentrates or compounds of the metal; or, in a 15 more specific aspect, to produce molybdenum or molybdenum compounds which may in themselves be the end of the process or from which the metal may be easily reduced in any of the several well known manners. 20 The general object of the invention is to produce or make it possible to produce the metal more inexpensively than is possible with present methods of which we are aware. There are also other minor objects of the 25 invention; but they will be best understood from the following specification wherein we describe preferred methods of procedure in accordance with and illustrative of our invention.

30 The particular method, illustrative of our invention, described in the following specification is particularly suitable for obtaining the metal from ores or compounds in which it is present as sulphides, oxides, or as molybdates such for instance as lead molybdate. The molybdates need not be roasted—they may be treated in that form. And where we have other compounds such as sulphides to work with we may either 35 roast to oxides or they may be fused with sodium carbonate (soda ash for instance) to produce a sodium molybdate. And the other molybdates, as lead molybdate, wulfenite, may be likewise treated with sodium 40 carbonate to get a sodium molybdate. In known ores the metal usually exists in the form of sulphide, and in some ores this is accompanied by appreciable amounts of oxides. The sulphide, molybdenite, can be 45 extracted readily as a concentrate by known methods; but the oxides cannot be extracted in this way and ores containing the oxides do not give a satisfactory recovery when treated by concentration. By our method

the oxidized compounds are readily extracted, either with or without preliminary concentration.

In order to give first a simple view of our process we shall suppose that we start with the sulphide, either concentrated or 60 in an ore. The steps are then briefly (and illustratively but not as a limitation) stated as follows:

1. Roasting the sulphide compounds to produce molybdenum oxide or oxides and 65 other compounds, for instance molybdenum sulphate; or

1a. Fusion with sodium carbonate to produce sodium molybdate.

2. Leaching the resulting compounds (at 70 the start of the process) in a solution to produce a sodium molybdate electrolyte and after the process is in operation leaching with depleted electrolyte; or

2a. (corresponding to "1a" above) leaching 75 from the fusion product with water or with acidulated water.

3. Electrolyzing the solution of molybdenum thus made to produce a molybdenum deposit at the cathode, and to regenerate 80 solution for re-use as solvent on fresh ore.

4. Further treatment of the cathode product if desired. Further details and ramifications of the process are explained herein-after.

In order to produce a satisfactorily complete roast we find it necessary to reduce the size of the molybdenum concentrates. Molybdenum concentrates as usually produced consist of lumps of such large size 90 that they cannot be roasted satisfactorily, since the oxidation results in the lumps becoming coated with a more or less impervious oxide coating which prevents access of air to the interior unroasted sulphide. 95 We have therefore found it necessary before roasting to reduce the sizes to such a degree that this result does not take place and so that the pieces will roast clear through. The roast is carried out from 760° 100 F. to 1040° F., these being approximately the temperatures within which oxidizing reaction of the sulphide takes place. When roasting unconcentrated ores extraneous heat may be required to maintain the roasting temperature; but in roasting commercial concentrates the heat of oxidation may be sufficient to keep up the roasting temper-

ature, or may even tend to carry the temperatures too high. During the period of oxidation the temperature should be kept as low as possible to avoid volatilization losses and must be kept below the sintering temperature of the oxides produced.

The resultant roasted product, under the conditions named, will have most of its molybdenum in the form of the trioxide 10  $\text{MoO}_3$  soluble in the leaching solution or depleted electrolyte whether alkaline, neutral or acid; and this is also true of the oxidized compounds usually originally present in ores.

15 Then in the second main step of our process, in starting operations, we leach out the roast preferably with an alkali solution (for instance, a solution of caustic soda). This solution is made of sufficient strength to react with the  $\text{MoO}_3$  to form sodium molybdate and further preferably to have a sufficient excess of  $\text{MoO}_3$  to form a final electrolyte that is distinctly acid by forming molybdic acid with the water of the solution. We 20 may in this process use a solution carrying any convenient percentage of molybdenum; we find that about  $2\frac{1}{2}\%$   $\text{MoO}_3$  is about as low as we care to go for commercially profitable operation and therefore we find it convenient to start with a solution of about 5% 25  $\text{MoO}_3$ . Consequently, as a matter of illustration, we will say here that we use a caustic solution strong enough to react with a quantity of calcine equivalent to the 5% of  $\text{MoO}_3$  to produce sodium molybdate and leave enough of the  $\text{MoO}_3$  to have a final 30 distinctly acid solution due to the excess of  $\text{MoO}_3$  forming molybdic acid with the water of the solution. Or free acid, as sulphuric, 35 may be added to get the desired acid condition. It may be desirable in some cases either to have a neutral solution or even to have a somewhat alkaline solution for the next succeeding step of electrolysis; as we 40 find we are able by having a neutral or alkaline solution to produce other compounds that may be desirable. The acidity, alkalinity, or neutrality of the electrolyte may be controlled by properly proportioning the 45 amounts caustic and  $\text{MoO}_3$ , as will readily be understood. By control of this solution we may more or less control the nature of the electrolytic deposit, to produce molybdenum, or oxides, or other compounds. However, 50 in general we preferably use a distinctly acid solution. We find that a small percentage of free acid also prevents co-precipitation of some impurities, as sodium. We find about 2.5% total acidity to give good results 55 in the electrolysis.

60 We may also treat the sulphide directly to form a water soluble alkali-molybdate. Thus we may fuse the sulphide with soda ash to produce a mass containing sodium molybdate and then leach out the mass with

water or acidulated water to get a solution of sodium molybdate. Likewise we may treat other molybdates in the same manner. When we treat for example wulfenite ores or concentrates the product resulting from the fusion with soda ash is leached with water, (or may be leached with regenerated depleted electrolyte as hereinafter explained) leaving in the residue lead, copper, gold, silver and other substances, which residue may be treated separately for other values. The water solution of sodium molybdate obtained by treating the fusion mass may be adjusted as to acidity as explained above by the addition of free sulphuric acid. 70

75 It will be understood that the leaching operation and the separation of the solution from the gangue may be accomplished in any suitable apparatus. After the initial starting of the process, in which a freshly prepared solution is used, the leaching solution is provided by operation of the process itself, as will later be understood, and so this leaching solution as used in the average run of the process will contain a certain percentage of molybdenum as we do not, in the next step of electrolysis, aim commercially to take out all of the metal. 80

85 Then in the next step of the process by electrolytic action we precipitate the dissolved metal at the cathode as sesquioxide or other form of molybdenum or molybdenum compound. The electrolysis may be carried out in any suitable electrolytic apparatus as in an ordinary electrolytic cell, 90 using an insoluble anode. Lead or graphite may be used as anode material. The cathode may be made of any one of several substances; for example, sheet iron or aluminum do very well. It is possible in this step to remove all of the metal, but not economical to do so by continued electrolysis; so we prefer to stop the electrolytic action when the solution reaches about  $2\frac{1}{2}\%$   $\text{MoO}_3$ . Operating between 5% and  $2\frac{1}{2}\%$   $\text{MoO}_3$  gives a 95 good average yield per unit of power. The current densities may be varied but we have found about 1.8 amperes per square foot of cathode surface to be a satisfactory density for practical use: We have also found that by 100 heating the electrolyte to about  $160^{\circ}$  F. it is possible to obtain an average precipitate yield of about  $1\frac{1}{2}$  to 2 lbs. per kilowatt hour as against a yield of about  $\frac{1}{2}$  lb. if the solution is not heated. Under these operating conditions the cathode deposit consists of molybdenum oxides and may contain other compounds of the metal, and the metal itself, but is usually mainly hydrated molybdenum sesquioxide. There may be small 105 amounts of other forms of molybdenum and small amounts of other substances also precipitated, depending upon what is present in the electrolyte. This deposit adheres to the cathode; but by removing and drying 110

by heating the cathode and its deposit we find the deposit to be readily removable. Thus for continuous operation we may remove the cathodes when they have a sufficient deposit and substitute fresh cathodes in their place while the removed ones are being dried and cleaned. If any of the deposit becomes detached from the cathode in the electrolytic cell, then this deposit may be readily separated by filtration or otherwise from the electrolyte before its subsequent use for leaching.

Going back now to the first part of our process we will explain certain variational and additional steps that may be used. For instance, ores that carry the metal as lead molybdate do not need to be roasted but may be treated as described above to produce sodium molybdate; the result being the solution of the molybdenum as sodium molybdate, and leaving the lead and other valuable constituents in the residues. In this connection we may point out one valuable feature of our process; that the presence of some other metals, objectionable in known molybdenum processes, is not objectionable in our process. For instance, ores, carrying copper are objectionable in ordinary methods, but are not objectionable in our method. All or most such metals are left in the gangue or are otherwise taken care of at the time of leaching.

In order to remove iron and some other metals that may be objectionable in some cases, we may first leach the calcine with water or acidulated water (say 1½% acid). After this leaching, the residue, being the remainder of the calcine that does not go into the water or acidulated water leaching solution, then is leached with depleted electrolyte as previously described. If the solution obtained by preliminary leaching contains appreciable amounts of molybdenum, it may be treated in known ways (for instance, treatment with an alkali such as caustic soda, or sodium carbonate) to remove iron and then be added to the main solution for electrolysis.

Before electrolyzing the sodium molybdate solution we may heat and filter it to remove any suspended impurities.

In the step of electrolysis the molybdenum is deposited at the cathode in the form of molybdenum or oxides and the solvent is also regenerated. This regenerated solution then goes back into the process, being used to leach more of the calcine, or the residue of the calcine as above explained; or is joined with the water or acid solution resulting from the preliminary sodium carbonate treatment of the ores or concentrates, as above explained; or is used to leach out the fusion mass instead of the water or acidulated water as explained above. In this last mentioned case we may neutralize

the regenerated depleted electrolyte, if necessary, before leaching, to obviate the possibility of acid present in the leaching solution taking any undesirable impurities out of the mass being leached. Thus the use of the leaching solution is cyclical; and the solution having been once made up it is only necessary thereafter to add caustic or acid to the process to make up a casual deficiency, or to add some fresh solution to make up for the discard of a small part of the solution each cycle to prevent building up of undesirable impurities. Of course the total or free acidity of the electrolyte diminishes as the MoO<sub>3</sub> is removed in the electrolyzing step; but the acidity is renewed when new calcine is leached with the depleted electrolyte or when it is joined with the leach solution from the fusion operation, as before described.

We have stated that we prefer to use an acid electrolyte. We find that production is greater from an acid electrolyte than from a neutral or alkaline one, but find that it is possible to produce a molybdenum deposit even with an electrolyte distinctly alkaline. However we find that the nature of the deposit varies with, and to a certain extent can be controlled by, the degree of acidity or alkalinity of the electrolyte; and so, although the acid electrolyte is preferred for maximum deposit, we do not wish to limit our process specifically or entirely to an acid electrolyte.

The sesquioxide (Mo<sub>2</sub>O<sub>5</sub>) or other compounds as detached from the cathode may be marketed in that form or may be used for the production of the metal or compounds of the metal. For the production of metallic molybdenum, the sesquioxide which we produce has very considerable advantages. So far as we are aware the sesquioxide has never been commercially used for production of the metal. In comparison with the trioxide which has ordinarily been used for production of the metal the sesquioxide requires theoretically only one half the amount of reducing agent; and this is an important feature of practical economy where hydrogen is used or where the reduction is by alumino-thermic methods.

As the last step of the process—the reduction of the cathode products to metal,—we do not make any specific claim in itself, but we prefer to use hydrogen as the reducing agent, and the operation may be carried on in any suitable apparatus. The result of reduction of the cathode products is a finely divided powder, which can be reduced to solid form in various manners not necessary here to specify.

Having described a preferred form of our invention, we claim:

1. The process for extracting molybdenum from concentrates and ores, that in-

cludes roasting to convert sulphide compounds into oxides, then treating the calcine with dilute sulphuric acid to remove impurities, then treating the residue from the acid treatment to form an acid solution of sodium molybdate, then warming the resulting solution and electrolyzing it to precipitate molybdenum compounds at the cathode and to regenerate the depleted electrolyte for reuse as a solvent; then drying, dehydrating, and removing the deposit from the cathode.

2. The process for extracting molybdenum from concentrates and ores, that includes roasting to convert sulphide compounds into oxides, then treating the calcine with dilute sulphuric acid to remove impurities, then separating such impurities from the resulting solution, then treating the residue from the acid treatment to form an acid solution of sodium molybdate, then warming the resulting solution and electrolyzing it together with the solution resulting from the first leaching to precipitate molybdenum compounds at the cathode and to regenerate the depleted electrolyte for reuse as a solvent; then drying, dehydrating, and removing the deposit from the cathode.

3. The process for extracting molybdenum from concentrates and ores, that includes roasting to convert sulphide compounds into oxides, then treating the calcine with dilute sulphuric acid to remove impurities, then treating the residue from the acid treatment with a depleted electrolytic solution, then separating the gangue from the solution, then warming the resulting solution and electrolyzing it to precipitate molybdenum compounds at the cathode and to regenerate the depleted electrolyte for reuse as a solvent; then drying, dehydrating, and removing the deposit from the cathode.

4. The process for extracting molybdenum from concentrates and ores that includes forming a solution of an alkali-molybdenum compound, then warming the solution and electrolyzing it to produce a molybdenum deposit and to regenerate the depleted electrolyte for reuse as a solvent, and then using the regenerated solution for the formation of more solution of alkali-molybdenum compound for continued practice of the process.

5. The process for extracting molybdenum from concentrates and ores that includes forming a solution of an alkali-molybdenum compound, with a definite total acidity, then warming the solution and electrolyzing it to produce a molybdenum deposit and to regenerate the depleted electrolyte for reuse as a solvent, and then using the regenerated solution for the formation of more solution of alkali-molybdenum compound for continued practice of the process.

6. The process for extracting molybdenum from concentrates and ores, that includes conversion of sulphide compounds into oxides, then (to initially start the process) dissolving the oxides in a sodium hydroxide solution to form a sodium molybdate solution with an excess of the oxides to form free molybdcic acid to give the solution a free acidity; then electrolyzing the solution to precipitate molybdenum compounds at the cathode and to regenerate the depleted solution for further use as a solvent; and then using the regenerated solvent to dissolve further oxides for the continued practice of the process, the acidity of the electrolyte being maintained at each dissolving operation by the use of an excess of the oxides.

7. The process for extracting molybdenum from concentrates and ores, that includes conversion to a soluble alkali-molybdate and the formation of a solution of the molybdate, said solution having a free acidity, then electrolyzing the solution to precipitate molybdenum compounds at the cathode and to regenerate the depleted electrolyte for reuse as a solvent, then using the regenerated solvent to form more solution of the alkali molybdate for the continued practice of the process, maintaining at each solution operation the free acidity of the solution.

8. The process for extracting molybdenum from concentrates and ores, that includes the conversion of sulphides into oxides, then treating the calcine with dilute sulphuric acid to remove impurities, separating the impurities from the resulting solution, treating the residue from the acid treatment with an alkali solution to form an alkali-molybdate solution, the oxides being used in excess to give the solution a free acidity by the formation of molybdcic acid, then separating said solution from the gangue, warming the solution and electrolyzing it together with the solution resulting from the sulphuric acid treatment to precipitate molybdenum compounds in the cathode and to regenerate the depleted electrolyte for reuse as a solvent, then using the regenerated solvent to dissolve more of the oxides, maintaining the free acidity of the solution at each dissolving operation.

9. The process of treating molybdenum oxides soluble in an alkali solution, that includes dissolving the oxides in an alkali solution to produce an alkali-molybdate solution, the oxide being used in excess to form free molybdcic acid to make the solution definitely acid; and then electrolyzing the resultant solution.

10. The process of treating molybdenum oxides soluble in an alkali solution, that includes dissolving the oxides in an alkali solution to produce an alkali-molybdate

solution, the oxides being used in excess to form free molybdcic acid to make the solution definitely acid; then electrolyzing the resultant solution to produce a cathode product and to regenerate the depleted electrolyte for reuse as a solvent, and then using the regenerated solution to dissolve more of the oxides for continued practice of the process, the acidity being maintained by use of an excess of the oxides.

11. The process for extracting molybdenum from concentrates and ores, that includes treatment with sodium carbonate to form sodium molybdate, forming a solution of the molybdate, electrolyzing the solution to produce a cathode product and to regenerate the depleted electrolyte for further use in the process, and then using the regenerated solution to dissolve more sodium molybdate in the continued practice of the process.

12. The process for extracting molybdenum from concentrates and ores, that includes fusion of a molybdate carrying ore or concentrate with sodium carbonate to form a mass containing sodium molybdate,

leaching the mass to form a solution of sodium molybdate, then electrolyzing the solution to produce a cathode product and to regenerate the depleted solution for further use.

13. The process for extracting molybdenum from concentrates and ores that includes forming a solution of an alkali-molybdenum compound, then electrolyzing the solution to produce a molybdenum deposit and to regenerate the depleted electrolyte for reuse as a solvent, and then using the regenerated solution for the formation of more solution of alkali-molybdenum compound for continued practice of the process.

In witness that we claim the foregoing we have hereunto subscribed our names this 27th day of October, 1922.

GEORGE D. VAN ARSDALE.

RUSH T. SILL.

HARLEY A. SILL.

Witnesses:

W. E. HAYES,  
ARTHUR K. LOSSNER,  
S. J. MAY.